

1

3,441,404

## EXTRACTION OF COPPER FROM MOLTEN METAL MELTS

Kenneth H. Ivey, Adelphi, Md., and Sidney J. Chastain, Knoxville, Tenn., assignors to the United States of America as represented by the Secretary of the Interior  
No Drawing. Filed Nov. 25, 1966, Ser. No. 597,162  
Int. Cl. C22b 15/00

U.S. Cl. 75—76

10 Claims

### ABSTRACT OF THE DISCLOSURE

Removing copper from molten scrap iron by adding sulfur and halide-containing compound to the melt whereby resultant halide vapor strips off copper-sulfur compound.

This invention relates to the removal of copper in the reclamation of metal scrap.

For some years now, the United States has imported large quantities of iron ore since foreign ore possesses higher quality than domestic ore and can be delivered at competitive costs. While there are large domestic supplies of scrap iron available in junk cars, it is considered unusable as clean basic cast iron because copper, in the form of small wires and tubing, is not removed by the junk dealer for economic reasons. When this scrap is melted, the ingot contains enough copper to cause the metal to be unusable as a source material for metallurgical industries.

It has now been discovered that copper can be removed from such metals by treating it in a molten state with sulfur and a halide-containing compound selected from the group consisting of alkali earth metal halides, alkali metal halides, alkali earth metal silicohalides, alkali metal silicohalides,  $\text{KMgF}_3$ ,  $\text{KAIF}_4$ ,  $\text{K}_2\text{TiF}_6$ ,  $\text{K}_2\text{ZrF}_6$  and  $\text{K}_2\text{SnF}_6$ . One theory advanced with regard to the process is that the sulfur forms copper sulphide with copper in the metal, and the halide vaporizes and strips off the sulphide.

Therefore, it is an object of this invention to provide a method for the removal of copper from metal melts.

Another object is to provide cast iron and other metals free of copper.

A further object is the introduction of materials having a low vapor pressure into a bath of molten metal whereby the danger of explosion is eliminated.

A still further object is the introduction of a volatile material into a bath of molten metal, whereby the volatile material helps to free copper from the metal melt.

Other objects and advantages will be obvious from the detailed description of the process appearing in the specification.

In the practice of this invention, the halide-containing compound is mixed with sulfur to form the treating agent, and the agent combined with the copper-containing molten metal by (1) placing the agent in the bottom of the furnace or crucible prior to melting the metal; or (2) adding the agent to the molten metal; or (3) pouring the molten metal into a ladle containing the agent. When the agent contacts the molten metal, heavy fumes containing the copper are given off. After the fuming ceases, the molten mass can be cast or poured. An easily removable slag, which contains elements from the agent, forms on top of the resultant ingot. After slag removal, the ingot, substantially free of copper, can be worked in the conventional manner.

To obtain substantial removal of the copper, sulfur is preferably added in amounts ranging from about 2 to about 6 parts per part of copper; the halide-containing

2

compound being added in amounts ranging from about 4 to about 8 parts per part of sulfur. If lesser amounts of treating agent are employed, smaller percentages of copper will be removed.

5 The following examples illustrate the effectiveness of the process of the present invention:

### EXAMPLE I

Cast iron, copper and the treating agent were used in the following percentages:

|                             | Grams |
|-----------------------------|-------|
| 10 Cast iron                | 45    |
| Copper metal                | 5     |
| 15 $\text{K}_2\text{SiF}_6$ | 30    |
| Sulfur                      | 10    |

The potassium silicofluoride and sulfur were placed in the bottom of a graphite crucible; the cast iron mixed with the copper was placed on top of the treating agent. The crucible was then placed in a furnace and the mixture 20 melted. Once fuming had ceased, the melt was removed from the furnace and a button was cast.

Results.—On cooling, the slag was removed from the metal button which was cut into sections, and the shavings were analyzed. The analysis gave the following results:

|       | Percent           |
|-------|-------------------|
| 30 K  | 0                 |
| Ca    | 0                 |
| Ti    | .1                |
| V     | 0                 |
| 35 Cr | .3                |
| Fe    | Major constituent |
| Ni    | .1                |
| Cu    | .2                |

35 These data indicates that 98 percent of the copper was removed from the metal melt during the process.

### EXAMPLE II

|                          | Grams |
|--------------------------|-------|
| 40 Sulfur used           | none  |
| Cast iron                | 45    |
| Copper metal             | 5     |
| $\text{K}_2\text{SiF}_6$ | 30    |

45 The object was to test only potassium silicofluoride as a treating agent. The materials were treated and processed as in Example I. After melting and cooling was completed, the sample was prepared for analysis.

Results.—Spectrographic analysis showed that only 50 percent of the copper was removed by this method, pointing up the fact that sulfur is an important component of the process.

### EXAMPLE III

55 In this example only sulfur was used as a treating agent.

|              | Grams |
|--------------|-------|
| Cast iron    | 45    |
| Copper metal | 5     |
| Sulfur       | 30    |

60 The materials were prepared, melted, and poured in the same manner as the above examples.

65 Results.—Spectrographic analysis indicated only about 40 percent of the copper was removed; thus, pointing up the fact that alkali silicofluoride is an important component of this process.

As shown in the above examples, if the halide-containing compound or the sulfur are used alone, only part of the copper is removed. In other tests when larger amounts of the halide-containing compound or sulfur were used alone, no appreciable increase in the amount of copper removal was indicated. However, when used

in combination, larger amounts of these agents remove greater amounts of copper.

Besides the fluorides, other halides such as alkali and alkali earth metal chlorides and bromides are effective copper removal agents.

Copper can substantially be removed by the process of the present invention from ferrous metals such as scrap iron and alloy steels containing up to as much as about 30% copper by weight. Furthermore, by the process, junked cars which present a disposal problem and even larger stockpiles of other scrap metal would be available for reprocessing. Any of the furnacing techniques now used by the industry could be employed. Finally, the removed copper composition could be recovered by, for example, filtering or washing the gas or fumes, or by any other conventional method.

Although the particular process herein described is well adapted to carry out the objects of the present invention, it is to be understood that various modifications and changes may be made all coming within the scope of the following claims.

What is claimed is:

1. A process for removing copper from a copper-containing ferrous metal comprising reacting the said copper-containing ferrous metal while in a molten state with sulfur and a halide-containing compound selected from the group consisting of alkali metal halides, alkali earth metal halides, alkali metal silicohalides, alkali earth metal silicohalides,  $KMgF_3$ ,  $KAlF_4$ ,  $K_2TiF_6$ ,  $K_2ZrF_6$  and  $K_2SnF_6$ , to strip said copper from said copper-containing ferrous metal.

2. The process of claim 1 wherein said halide-containing compound is a fluoride-containing compound.

3. The process of claim 1 wherein said halide-containing compound is potassium silicofluoride.

4. The process of claim 1 wherein said reaction step comprises mixing said molten metal with sulfur and said halide-containing compound.

5. The process of claim 4 wherein said halide-containing compound is a fluoride.

6. The process of claim 4 wherein said halide-containing compound is potassium silicofluoride.

7. The process of claim 4 wherein said metal contains less than about 30% by weight copper, and wherein said sulfur is added in an amount ranging from about 2 to about 6 parts per part of copper present in said metal, and said halide-containing compound is added in an amount ranging from about 4 to about 8 parts per part of sulfur added.

15 8. The process of claim 1 wherein said metal is scrap iron.

9. The process of claim 2 wherein said metal is scrap iron.

10 10. The process of claim 3 wherein said metal is scrap iron.

#### References Cited

##### UNITED STATES PATENTS

|    |           |         |       |          |
|----|-----------|---------|-------|----------|
| 25 | 393,258   | Beck    | ----- | 110—85   |
|    | 2,362,202 | Hay     | ----- | 23—135 X |
|    | 2,403,419 | Wilkins | ----- | 75—44    |
|    | 2,662,009 | Roberts | ----- | 75—108   |
|    | 2,683,085 | Lohberg | ----- | 75—63    |

30 L. DEWAYNE RUTLEDGE, *Primary Examiner.*

J. E. LEGRU, *Assistant Examiner.*

U.S. Cl. X.R.

35 23—135; 75—44, 63